# EUROPEAN PATENT SPECIFICATION

(11) **EP 3 225 359 B1**
(45) Date of publication and mention of the grant of the patent: **09.01.2019**
(21) Application number: 15909578.5
(22) Date of filing: 09.12.2015
(51) Int. Cl.: B22C 9/02, B22D 19/00, B22D 19/06, C22C 1/10, C22C 29/16, C23C 6/00, B24C 5/04

(54) **METHOD FOR PREPARING SHOT FLOWING PIPE OF COMPOSITE SHOT BLASTING MACHINE**
VERFAHREN ZUR HERSTELLUNG EINES STRAHLSTRÖMUNGSROHRS EINER KOMPOSITKUGELSTRAHLMASCHINE
PROCÉDÉ DE PRÉPARATION DE TUBE D'ÉCOULEMENT DE GRENAILLE POUR UNE MACHINE DE GRENAILLAGE COMPOSITE

(30) Priority: 03.12.2015 CN 201510876689
(43) Date of publication of application: 04.10.2017
(73) Proprietor: Shandong Kaitai Shot Blasting Machinery Share Co., Ltd, Binzhou, Shandong 256217 (CN)
(72) Inventor: WANG, Shouren, Ji'nan Shandong 250022 (CN); LI, Yadong, Ji'nan Shandong 250022 (CN); WANG, Ruiguo, Binzhou Shandong 256217 (CN); ZHANG, Xiao, Binzhou Shandong 256217 (CN); ZHANG, Laibin, Binzhou Shandong 256217 (CN); WU, Chengmin, Binzhou Shandong 256217 (CN)
(74) Representative: Sun, Yiming
(86) International application number: PCT/CN2015/096787
(87) International publication number: WO 2017/092064

(56) References cited:
- EP-A2- 1 256 403
- CN-A- 101 565 308
- CN-A- 102 021 469
- CN-A- 102 703 851
- CN-A- 103 817 607
- CN-U- 201 881 277
- DE-A1- 3 528 137
- GB-A- 1 479 589
- JP-A- H10 246 233
- RU-U1- 106 580
- US-A- 3 608 170

## Description

### Technical Field

The present invention relates to the technical field of preparation of a shot flowing tube (spout) of a shot blasting device (SBM), in particular to a preparing method of a composite shot flowing tube (spout) of the shot blasting device (SBM).

### Related Art

Along with the continuous development of the industry, in the technical field of surface treatment, the application of the shot blasting technology to the current industry production is very wide, and the device used by the shot blasting technology is a shot blasting machine (SBM). The SMBis a treatment technology of blasting steel grit and steel shot at a high speed to impact onto the surfaces of materials and articles through a shot blasting device. It is used for removing burrs and iron rust on the surface of a workpiece, it can also remove pollutants on the surface of specific parts of the coating of the workpiece. Furthermore it provides a surface profile which increases the adhesion of the coating, thereby improving the quality and durability of the workpiece. When compared with other surface treatment technologies it has the advantages of higher speed and higher efficiency.

One of the core components in the SBMis the blast wheel. When the SBM is in operation the steel grit and steel shot enter the control cage through a shot flowing tube (spout), before being accelerated by centrifugal force by a rotary blast wheel and impacting onto the surface of the workpiece to achieve the aim of cleaning or strengthening.

During operation the shot continuously flowsthrough the SBM causing the component parts to experience wear.The spout of the SBM is subject to a high level of wear,therefore improving the durability and wear resistance of the spout would result in an increase in the life span and reliability of the SBM.

The spout in the current industrial production is made of a cast iron material, in long term use, due to the continuous high speed flow of the steel shot and steel grit, the spoutbecomes worn very quickly, and since the SBM is unable to operate, the production efficiency is greatly reduced, the production cost is increased, and financial loss is caused.

Ceramic is an ideal material to substitute for the traditional cast iron spout due to its properties: light weight, high pressure resistance, excellent wear resistance, etc. But currently ceramic spouts are not available - there is an urgent need for a composite spout with excellent performance to be used in SBM.

DE 35 28 137 A1 discloses a mouthpiece of a spray nozzle and a method for its manufacture. The mouthpiece of a spray nozzle consists of a moulding and of a protective casing surrounding the latter. The moulding is produced from a ceramic material of high wear resistance. The protective casing consists of a shock-proof and impact-resistant material elastic relative thereto and can be an iron sheet.

### Summary

In order to overcome the inherent weaknesses and shortcomings of the cast iron spouts used in existing SBM, the present invention provides a preparation method for a composite spout, which is simple and quick to manufacture, easy to operate and offers excellent performance.

The present invention is realized by the following technical manufacturing process:
The preparation method for a composite spoutto be used in SBM comprises of the following steps:
(1) Preparation of raw materials:
   - 80-85 parts by weight of silicon nitride powder
   - 5-10 parts by weight of boron nitride nanotube powder
   - 4-6 parts by weight of aluminum oxide powder
   - 3-5 parts by weight of yttrium oxide powder respectively
(2) Mixing of raw materials
   - add the raw materials in step (1) into a ball milling tank
   - add alcohol according to a volume ratio of alcohol to rawmaterials of 1:1
   - add steel shot according to a mass ratio of the steel shot to raw materials of 9-15:1
   - seal the ball milling tank
   - introduce argon gas into the ball milling tank as a protective gas
   - ball-milling and mixing the raw materials in a planetary ball mill
   - set the ball-milling rotary speed to be 200-250 rpm
   - the ball-milling duration is 8-12h
   - dry the ball-milled raw materials for 10-12h in a vacuum drying box
   - set the temperature to 75-85°C
   - pass the mixed materials after the drying through a 300-mesh sieve
   - collect the resulting material
(3) Preparation of slurry:
   - add the mixed materials obtained in step (2) into a stirring machine
   - add distilled water with a mass percent of 28-35%
   - add a diluent with a mass percent of 0.3-0.5%
   - stir the raw materials at a rotary speed of 250-300r/min for a duration of 1-2h
(4) Grouting molding:
   - inject the slurry obtained in step (3) into a molding gypsum die for the spout
   - pour excessive slurry in the die after a slurry layer is thickened to 10mm
   - centrifuge the model with a blank after the slurry is poured
(5) Drying demoulding:
   - place the model with a blank obtained in step (4) into a drying room with the temperature controlled at 53+/-3°C
   - demould the model with a blank after a grouting opening is separated from the blank by 0.5-1mmto obtain a blank of the shot flowing tube
(6) Vacuum sintering:
   - place the blank of the spout obtained in step (5) in a die of the spout
   - place into a vacuum thermal pressing sintering furnace with a vacuum degree of 10⁻²Pa
   - control the temperature rising process:
   - manually heating to 200°C
   - heating to 1100°C at a temperature rising rate of 10°C/min
   - maintain temperature for 30min
   - heat to 1750-1800°C at a rate of 7°C/min
   - end the sintering after maintaining temperature for 1h
   - this results in a Si₃N₄/BNNT composite ceramic liner of the spout after theworkpiece is cooled to room temperature in the furnace
(7) Composite casting:
   - load the Si₃N₄/BNNT composite ceramic liner of the spout obtained in step (6) into a casting sandbox of the spout
   - pour with molten iron after die assembly to wrap an iron casting onto the outer wall of the ceramic spout
   - this results in the composite spout of the SBM with outer side of cast iron and the inside of Si₃N₄/BNNT composite ceramic

The present invention has the characteristics:
The diluent in step (3) is one or combination of more of water glass or sodium carbonate or sodium phosphate or sodium hexametaphosphate; and the diluent is further preferably sodium carbonate.

The centrifuging the model with a blank after the slurry is poured in step (4) is to avoid uneven distribution of a little residual slurry on the inner surface of the blank after the slurry is poured, so as to ensure the uniform distribution of the residual slurry and avoid slurry strands.

The drying time for the model with a blank in step (5) is 2/5-3/5 of slurry charging time; further preferably, drying time for the model with a blank in step (5) is 1/2 of the slurry charging time.

The present invention has the beneficial effects:
In common with wearproof structure ceramics the silicon nitride ceramic has the advantages of:
- high strength
- high hardness
- high temperature resistance
- wear resistance
- corrosion resistance
- oxidation resistance
- good thermal shock resistance
- high density

The boron nitride nanotubes feature the following properties:
- chemical stability
- excellent mechanical properties
- heat conductivity
- low thermal expansion
- excellent oxidation resistance

Silicon nitride also reduces the brittleness of a silicon nitride ceramic product and improves the crack growth resistance after composite with the silicon nitride ceramic material, and thus becomes an ideal high-tenacity ceramic material for manufacturing the spout to be used in the SBM.

### (1) High hardness

The new Si₃N₄/BNNT composite ceramic material as mentioned in the present invention has very high hardness which is up to HRA94, and if the ceramic material is taken as the liner of the spout of the SBM, the hardness of the existing pure cast iron material is greatly improved, and greater durability in actual production use is realized.

### (2) Good wear resistance

The new Si₃N₄/BNNT composite ceramic material as mentioned in the present invention has very good wear resistance, the average friction coefficient is 0.285, and if the ceramic material is taken as the liner of the spout of the SBM, the wear resistance of the existing pure cast iron material is greatly improved, and the rejection rate of the spout is reduced.

### (3) Simple operation

All devices used in the preparation are common devices in a laboratory or production company, the operation process is simple and convenient and does not require sophisticated conditions or preparation.

In general, the preparation method of the present invention is simple and quick, the produced spoutfeaturing a Si₃N₄/BNNT composite ceramic material liner and a cast iron jacket integrates advantages of the ceramics and cast iron, thereby improving the hardness and wear resistance of the spout, reducing the weight of the product and meeting the requirements of industrial production.

### Detailed Description

The present invention is further explained in combination with the embodiments, but the present invention is not limited to specific examples herein.

### Embodiment 1:

(1) Raw material preparation:
   - 80 parts by weight of silicon nitride powder
   - 10 parts by weight of boron nitride nanotube powder
   - 5 parts by weight of aluminum oxide powder
   - 5 parts by weight of yttrium oxide powder respectively
(2) Raw material mixing:
   - (1) add the raw materials in step (1) into a ball milling tank
   - add alcohol according to a volume ratio of alcohol to raw materials of 1:1
   - add steel shot according to a mass ratio of steel shot to raw materials of 10:1
   - seal the ball milling tank
   - introduce argon gas into the ball milling tank as a protective gas
   - ball-mill and mix the raw materials in a planetary ball mill
   - set the ball-milling rotary speed to be 250 rpm
   - ball-milling time to be 10h
   - dry the ball-milled raw materials for 10h in a vacuum drying box
   - set the temperature into 75°C;
   - pass the mixed materials after the drying through a 300-mesh sieve
(3) Slurry preparing:
   - add the mixed materials obtained in step (2) into a stirring machine
   - add distilled water with a mass percent of 30%
   - add water solution with a mass percent of 0.3%
   - stir the raw materials at a rotary speed of 250r/min for a duration of 1h
(4) Grouting molding:
   - inject the slurry obtained in step (3) into a molding gypsum die for the spout
   - pour excessive slurry in the die after a slurry layer is thickened to 10mm
   - centrifuge the model with a blank after the slurry is poured
(5) Drying demoulding:
   - place the model with a blank obtained in step (4) into a drying room of which the temperature is controlled at 53+/-3°C
   - demould the model with a blank after a grouting opening is separated from the blank by 1mm to obtain a blank of the spout
   - the drying time of the model with a blank is 3/5 of the slurry charging time
(6) vacuum sintering:
   - place the blank of the spout obtained in step (5) in a die of the spout
   - place into a vacuum thermal pressing sintering furnace for vacuum hot pressing sintering at a vacuum degree of 10⁻²Pa
   - the temperature rising process consists of:
   - manually heating to 200°C
   - heating to 1100°C at a rate of 10°C/min
   - maintain temperature for 30min
   - heat to 1750°C at a rate of 7°C/min
   - maintain temperature for 1h
   - this results in a Si₃N₄/BNNT composite ceramic liner of the spout after theworkpiece is cooled to room temperature in the furnace
(7) Composite casting:
   - load the Si₃N₄/BNNT composite ceramic liner of the spout obtained in step (6) into a casting sandbox of the spout
   - pour in molten iron after die assembly to wrap an iron casting onto the outer wall of the ceramic spout
   - this results in the production of the composite spout of the SBM with outer side of cast iron and the inside of Si₃N₄/BNNT composite ceramic.

### Embodiment 2:

(1) Raw material preparation:
   - 82 parts by weight of silicon nitride powder
   - 8 parts by weight of boron nitride nanotube powder
   - 6 parts by weight of aluminum oxide powder
   - 4 parts by weight of yttrium oxide powder
(2) Mixing raw materials:
   - add the raw materials in step (1) into a ball milling tank
   - add alcohol according to a volume ratio of alcohol to raw materialsof 1:1
   - add steel shot according to a mass ratio of steel shot to raw materials of 9:1
   - seal the ball milling tank
   - introduce argon gas into the ball milling tank as a protective gas
   - ball-mill and mix the raw materials in a planetary ball mill
   - set the ball-milling rotary speed to 250 rpm for a duration of 8h
   - dry the ball-milled raw materials for 12h in a vacuum drying box
   - set the temperature into 85°C
   - pass the mixed materials after drying through a 300-mesh sieve
(3) Slurry preparation:
   - add the mixed materials obtained in step (2) into a stirring machine
   - add distilled water with a mass percent of 32%
   - addsodium carbonate with a mass percent of 0.4%
   - stir the raw materials at a rotary speed of 250r/min for 1.5h
(4) Grouting molding:
   - inject the slurry obtained in step (3) into a molding gypsum die for the spout of the SBM
   - pour excessive slurry in the die after a slurry layer is thickened to 10mm
   - centrifuge the model with a blank after the slurry is poured
(5) Drying demoulding:
   - place the model with a blank obtained in step (4) into a drying room at 53+/-3°C
   - demould the model with a blank after a grouting opening is separated from the blank by 1mm
   - to obtain a blank of the spout, wherein the drying time of the model with a blank is 1/2 of the slurry charging time
(6) Vacuum sintering:
   - place the blank of the spout obtained in step (5) in a die of the spout
   - place into a vacuum thermal pressing sintering furnace with a the vacuum degree of 10⁻²Pa
   - the temperature rising process consists of:
   - manually heating to 200°C
   - heating to 1100°C at a rate of 10°C/min
   - maintain temperature for 30min
   - heat to 1780°C at a rate of 7°C/min
   - maintain the temperature for 1h
   - this results in a Si₃N₄/BNNT composite ceramic liner for the spout after theworkpiece is cooled to room temperature in the furnace
(7) Composite casting:
   - load the Si₃N₄/BNNT composite ceramic liner of the spout obtained in step (6) into a casting sandbox of the spout
   - pourmolten iron after die assembly to wrap an iron casting onto the outer wall of the ceramic spout
   - this results in the production of the composite spout of the SBM with outer side of cast iron and the inside of Si₃N₄/BNNT composite ceramic.

### Embodiment 3:

(1) Raw material preparation:
   - 85 parts by weight of silicon nitride powder
   - 5 parts by weight of boron nitride nanotube powder
   - 4 parts by weight of aluminum oxide powder
   - 3 parts by weight of yttrium oxide powder
(2) Raw material mixing:
   - add the raw materials in step (1) into a ball milling tank
   - add alcohol according to a volume ratio of alcohol to raw materials of 1:1
   - add steel shot according to a mass ratio of steel shot to raw materials of 15:1
   - seal the ball milling tank
   - introduce argon gas into the ball milling tank as a protective gas
   - ball-mill and mix the raw materials in a planetary ball mill
   - set the ball-milling rotary speed to 200 rpm for a duration of 12h
   - dry the ball-milled raw materials for 12h in a vacuum drying box
   - set the temperature to 75°C
   - pass the mixed materials after the drying through a 300-mesh sieve
(3) Slurry preparation:
   - add the mixed materials obtained in step (2) into a stirring machine
   - add distilled water with a mass percent of 35%
   - add a combination of sodium phosphate and sodium hexametaphosphate with a mass percent of 0.5% when the mass ratio of sodium phosphate to sodium hexametaphosphate is 1:1
   - stir the raw materials at a rotary speed of 300r/min for 1h
(4) Grouting molding:
   - inject the slurry obtained in step (3) into a molding gypsum die for the spout
   - pour excessive slurry in the die after a slurry layer is thickened to 10mm
   - centrifuge the model with a blank after the slurry is poured
(5) Drying demoulding:
   - place the model with a blank obtained in step (4) into a drying room of which the temperature is controlled at 53+/-3°C
   - demould the model with a blank after a grouting opening is separated from the blank by 1mm
   - the drying time of the model with a blank is 2/5 of the slurry charging time
(6) Vacuum sintering:
   - place the blank of the shot flowing tube obtained in step (5) in a die of the spout
   - place into a vacuum thermal pressing sintering furnace with a vacuum degree of 10⁻²Pa
   - the temperature rising process consists of:
   - manually heating to 200°C
   - heat to 1100°C at a rate of 10°C/min
   - maintain temperature for 30min
   - heat to 1800°C at a rate of 7°C/min
   - maintain temperature for 1h
   - this results in obtaining a Si₃N₄/BNNT composite ceramic liner of the spout after a workpiece is cooled to room temperature in the furnace
(7) Composite casting:
   - load the Si₃N₄/BNNT composite ceramic liner of the spout obtained in step (6) into a casting sandbox of the spout
   - pour with molten iron after die assembly to wrap an iron casting onto the outer wall of the ceramic spout
   - this results in the production of the composite spout of the SBM with outer side of cast iron and the inside of Si₃N₄/BNNT composite ceramic.

The comparison between performances of the composite shot flowing tube prepared by the three embodiments and those of the existing cast iron shot flowing tube is asshown in table 1.

**Table 1**

| Performance preparing method | Embodiment1 | Embodiment 2 | Embodiment 3 | Cast iron |
|---|---|---|---|---|
| Rockwell hardness | 92.5 | 94.8 | 93.8 | 48 |
| Density (g·cm⁻³) | 3.27 | 3.39 | 3.35 | 7.31 |
| wear rate under 40N load (×10⁻⁷cm³·m⁻¹) | 1.35 | 1.22 | 1.31 | 75 |
| wear rate under 100N load (×10⁻⁷cm³·m⁻¹) | 6.57 | 6.08 | 6.29 | 120 |

It can be known from the above table that compared with the existing cast iron spout, the composite spout prepared by the present invention has higher hardness and lower density, which causes the weight of the composite spout to be only half that of the cast iron spout having the same volume, but the hardness of the composite spout to be twice that of the cast iron spout. In respect of wear resistance, the wear rate of the composite spoutof present invention is much lower than that of the cast iron spout under the same load action, which indicates that the wear performance of the former is far superior to that of the latter, and in the above three embodiments, the spout obtained in embodiment 2 has the best performance, therefore, the preparing process in embodiment 2 is the optimal method for preparing the composite spout.

In conclusion, the composite spout of the SBM prepared according to the present invention adopts a molding technology of a water absorption gypsum die, and features the following characteristics:
- high strength
- good wear resistance
- light weight of the Si₃N₄/BNNT composite ceramic

Therefore, the hardness and wear resistance of the currently adopted pure cast iron spout are improved, the durability of the spout caused by the flowing of shot materials in the spout in a long-term use process is reduced, such that the rejection rate of the spout is greatly reduced, the production cost is saved, the production efficiency is improved and the composite spout is an excellent and innovative spout for use in SBM.

## Claims

1. The preparation method of a composite spout of a SBM comprising of the following steps:
(1) Raw material preparation:
- 80-85 parts by weight of silicon nitride powder
- 5-10 parts by weight of boron nitride nanotube powder
- 4-6 parts by weight of aluminum oxide powder
- 3-5 parts by weight of yttrium oxide powder
(2) Raw material mixing:
- add the raw materials in step (1) into a ball milling tank
- add alcohol according to a volume ratio of alcohol to raw materials of 1:1
- add steel shot according to a mass ratio of the steel shot to raw materials of 9-15:1
- seal the ball milling tank
- introduce argon gas into the ball milling tank as a protective gas
- ball-mill and mix the raw materials in a planetary ball mill with a rotary speed of 200-250 rpm and a duration of 8-12h
- dry the ball-milled raw materials for 10-12h in a vacuum drying box at a temperature of 75-85°C
- pass the mixed materials after the drying through a 300-mesh sieve
(3) Slurry preparation:
- add the mixed material obtained in step (2) into a stirring machine
- add distilled water with a mass percent of 28-35%
- add a diluent with a mass percent of 0.3-0.5%
- stir the raw materials at a rotary speed of 250-300r/min for 1-2h
(4) Grouting molding:
- inject the slurry obtained in step (3) into a molding gypsum die for the spout of the SBM
- pour excessive slurry in the die after a slurry layer is thickened to 10mm
- centrifuge the model with a blank after the slurry is poured
(5) Drying demoulding:
- place the model with a blank obtained in step (4) into a drying room at a temperature of 53+/-3°C
- demould the model with a blank after a grouting opening is separated from the blank by 0.5-1 mm
- this results in a blank of the spout
(6) Vacuum sintering:
- place the blank of the spout obtained in step (5) in a die of the spout
- place it into a vacuum thermal pressing sintering furnace with a vacuum degree of 10⁻²Pa
- the temperature rising process consists of:
- manually heating to 200°C
- heat to 1100°C at a rate of 10°C/min
- maintain temperature for 30min
- heat to 1750-1800°C at a rate of 7°C/min
- maintain temperature for 1h
- this results in a Si₃N₄/BNNT composite ceramic liner of the spout after a workpiece is cooled to room temperature in the furnace
(7) Composite casting:
- load the Si₃N₄/BNNT composite ceramic liner of the spout obtained in step (6) into a casting sandbox of the spout
- pour molten iron after die assembly to wrap an iron casting onto the outer wall of the ceramic spout, thus finally obtaining the composite spout of the SBM with outer side of cast iron and the inside of Si₃N₄/BNNT composite ceramic

2. The preparation method of a composite spout of a SBM according to claim 1, **characterized in that** the diluent in step (3) is one or combination of more of water glass or sodium carbonate or sodium phosphate or sodium hexametaphosphate.

3. The preparation method of a composite spout of a SBM according to claim 2, **characterized in that** the diluent is sodium carbonate.

4. The preparation method of a composite spout of a SBM according to claim 1, **characterized in that** the drying time for the model with a blank in step (5) is 2/5-3/5 of slurry charging time.

5. The preparation method of a composite spout of a SBM according to claim 4, **characterized in that** the drying time for the model with a blank in step (5) is 1/2 of the slurry charging time.

6. The preparation method of a composite spout of a SBM according to claim 1, comprising the steps in detail:
(1) Raw material preparation:
- 80 parts by weight of silicon nitride powder
- 10 parts by weight of boron nitride nanotube powder
- 5 parts by weight of aluminum oxide powder
- 5 parts by weight of yttrium oxide powder
(2) Raw material mixing:
- add the raw materials in step (1) into a ball milling tank
- add alcohol according to a volume ratio of alcohol to raw materials of 1:1
- add steel shot according to a mass ratio of steel shot to raw materials of 10:1
- seal the ball milling tank
- introduce argon gas into the ball milling tank as a protective gas
- ball-mill and mix the raw materials in a planetary ball mill at a rotary speed of 250 rpm with a duration of 10h
- dry the ball-milled raw materials for 10h in a vacuum drying box at a temperature of 75°C
- pass the mixed materials after drying through a 300-mesh sieve
(3) Slurry preparation:
- add the mixed material obtained in step (2) into a stirring machine
- add distilled water with a mass percent of 30%
- add water solution with a mass percent of 0.3%
- stir the raw materials at a rotary speed of 250r/min for 1h
(4) Grouting molding:
- inject the slurry obtained in step (3) into a molding gypsum die for the spout of the SBM
- pour excessive slurry in the die after a slurry layer is thickened to 10mm
- centrifuge the model with a blank after the slurry is poured
(5) Drying demoulding:
- place the model with a blank obtained in step (4) into a drying room at a temperature of 53+/-3°C
- demould the model with a blank after a grouting opening is separated from the blank by 1mm to obtain a blank of the shot flowing tube
- the drying time of the model with a blank is 3/5 of the slurry charging time
(6) Vacuum sintering:
- place the blank of the spout obtained in step (5) in a die of the spout
- place into a vacuum thermal pressing sintering furnace with a vacuum degree of 10⁻²Pa and a temperature rising process consisting of:
- manually heat to 200°C
- heat to 1100°C at a rate of 10°C/min
- maintain temperature for 30min
- heat to 1750°C at a rate of 7°C/min
- maintain temperature for 1h
- this results in obtaining a Si₃N₄/BNNT composite ceramic liner of the spout after a workpiece is cooled to room temperature in the furnace
(7) Composite casting:
- load the Si₃N₄/BNNT composite ceramic liner of the spout obtained in step (6) into a casting sandbox of the spout
- pour with molten iron after die assembly to wrap an iron casting onto the outer wall of the ceramic spout
- this results in obtaining the composite spout of the SBM with outer side of cast iron and the inside of Si₃N₄/BNNT composite ceramic.

7. The preparation method of a composite spout of a WBM according to claim 1, comprising the steps in detail:
(1) Raw material preparation:
- 82 parts by weight of silicon nitride powder
- 8 parts by weight of boron nitride nanotube powder
- 6 parts by weight of aluminum oxide powder
- 4 parts by weight of yttrium oxide powder
(2) Raw material mixing:
- add the raw materials in step (1) into a ball milling tank
- add alcohol according to a volume ratio of alcohol to raw materialsof 1:1
- add steel shot according to a mass ratio of steel shot to raw materials of 9:1
- seal the ball milling tank
- introduce argon gas into the ball milling tank as a protective gas
- ball-mill and mix the raw materials in the planetary ball mill at a rotary speed of 250 rpm for a duration of 8h
- dry the ball-milled raw materials for 12h in a vacuum drying box at a temperature of 85°C
- pass the mixed materials after drying through a 300-mesh sieve
(3) Slurry preparation:
- add the mixed material obtained in step (2) into a stirring machine
- add distilled water with a mass percent of 32%
- addsodium carbonate with a mass percent of 0.4%
- stir the raw materials at a rotary speed of 250r/min for 1.5h
(4) Grouting molding:
- inject the slurry obtained in step (3) into a molding gypsum die for the spout of the SBM
- pour excessive slurry in the die after a slurry layer is thickened to 10mm
- centrifuge the model with a blank after the slurry is poured
(5) Drying demoulding:
- place the model with a blank obtained in step (4) into a drying room at a temperature of 53+/-3°C
- demould the model with a blank after a grouting opening is separated from the blank by 1mm which results in a blank of the spout
- the drying time of the model with a blank is 1/2 of the slurry charging time
(6) Vacuum sintering:
- place the blank of the spout obtained in step (5) in a die of the spout
- place into a vacuum thermal pressing sintering furnace at a vacuum degree of 10⁻²Pa
- the temperature rising process consists of:
- manually heat to 200°C
- heat to 1100°C at a rate of 10°C/min
- maintain temperature for 30min
- heat to 1780°C at a rate of 7°C/min
- maintain the temperature for 1h
- this results in obtaining a Si₃N₄/BNNT composite ceramic liner of the spout after the workpiece is cooled to room temperature in the furnace
(7) Composite casting:
- load the Si₃N₄/BNNT composite ceramic liner of the spout obtained in step (6) into a casting sandbox of the spout
- pour with molten iron after die assembly to wrap an iron casting onto the outer wall of the ceramic spout
- this results inobtaining the composite spout of the SBM with outer side of cast iron and the inside of Si₃N₄/BNNT composite ceramic.

8. The preparation method of a composite spout of a SBM according to claim 1, comprising the steps in detail:
(1) Raw material preparation:
- 85 parts by weight of silicon nitride powder
- 5 parts by weight of boron nitride nanotube powder
- 4 parts by weight of aluminum oxide powder
- 3 parts by weight of yttrium oxide powder
(2) Raw material mixing:
- add the raw materials in step (1) into a ball milling tank
- add alcohol according to a volume ratio of alcohol to raw materials of 1:1
- add steel shot according to a mass ratio of steel shot to raw materials of 15:1
- seal the ball milling tank
- introduce argon gas into the ball milling tank as a protective gas
- ball-mill and mix the raw materials in a planetary ball mill with a rotary speed of 200 rpm for a duration of 12h
- dry the ball-milled raw materials for 12h in a vacuum drying box at a temperature of75°C
- pass the mixed materials after drying through a 300-mesh sieve
(3) Slurry preparation:
- add the mixed material obtained in step (2) into a stirring machine
- add distilled water with a mass percent of 35%
- add a combination of sodium phosphate and sodium hexametaphosphate with a mass percent of 0.5% and where the mass ratio of sodium phosphate to sodium hexametaphosphate is 1:1
- stir the raw materials at a rotary speed of 300r/min for a duration of 1h
(4) Grouting molding:
- inject the slurry obtained in step (3) into a molding gypsum die for the spout of the SBM
- pour excessive slurry in the die after a slurry layer is thickened to 10mm
- centrifuge the model with a blank after the slurry is poured
(5) Drying demoulding:
- place the model with a blank obtained in step (4) into a drying room at a temperature of 53+/-3°C
- demould the model with a blank after a grouting opening is separated from the blank by 1mm to obtain a blank of the spout
- the drying time of the model with a blank is 2/5 of the slurry charging time
(6) Vacuum sintering:
- place the blank of the spout obtained in step (5) in a die of the spout
- place into a vacuum thermal pressing sintering furnace where the vacuum degree is 10⁻²Pa
- the temperature rising process consists of:
- manually heat to 200°C
- heat to 1100°C at a rate of 10°C/min
- maintain temperature for 30min
- heat to 1800°C at a rate of 7°C/min
- maintain temperature for 1h
- this results in obtaining a Si₃N₄/BNNT composite ceramic liner of the shot flowing tube after a workpiece is cooled to room temperature in the furnace
(7) Composite casting:
- load the Si₃N₄/BNNT composite ceramic liner of the spout obtained in step (6) into a casting sandbox of the spout
- pour with molten iron after die assembly to wrap an iron casting onto the outer wall of the ceramic spout
- this results in obtaining the composite spout of the SBM with outer side of cast iron and the inside of Si₃N₄/BNNT composite ceramic.

## Patentansprüche

1. Herstellungsverfahren für einen Verbundstutzen einer SBM, umfassend die folgenden Schritte:
(1) Rohstoffaufbereitung:
- 80 bis 85 Gewichtsteile Siliziumnitridpulver
- 5 bis 10 Gewichtsteile Bornitrid-Nanoröhrenpulver
- 4 bis 6 Gewichtsteile Aluminiumoxidpulver
- 3 bis 5 Gewichtsteile Yttriumoxidpulver
(2) Rohstoffmischung:
- Zugeben der Rohstoffe aus Schritt (1) in einen Kugelmahlbehälter
- Hinzufügen von Alkohol gemäß einem Volumenverhältnis von Alkohol zu Rohstoffen von 1:1
- Hinzufügen von Stahlkies gemäß einem Massenverhältnis von Stahlkies zu Rohstoffen von 9:1 bis 15:1
- Verschließen des Kugelmahlbehälters
- Einleiten von Argongas in den Kugelmahlbehälter als Schutzgas
- Kugelmahlen und Mischen der Rohstoffe in einer Planetenkugelmühle mit einer Rotationsgeschwindigkeit von 200 bis 250 rpm, und einer Dauer von 8 bis 12 Std.
- Trocknen der kugelgemahlenen Rohstoffe für 10 bis 12 Std. in einem Vakuum-Trockner bei einer Temperatur von 75 bis 85 °C
- Passieren der gemischten Materialen durch ein 300-maschiges Sieb nach dem Trocknen
(3) Aufschlämmungszubereitung:
- Zugeben des gemischten Materials, das in Schritt (2) erhalten wurde, in ein Rührgerät
- Hinzufügen von destilliertem Wasser mit einem Massenanteil von 28 bis 35 %
- Hinzufügen von einem Verdünnungsmittel mit einem Massenanteil von 0,3 bis 0,5 %
- Rühren der Rohstoffe bei einer Rotationsgeschwindigkeit von 250 bis 300 rpm für 1 bis 2 Std.
(4) Vergussformung:
- Einspritzen der Aufschlämmung, die in Schritt (3) erhalten wurde, in eine Formteilgipsmatrize für den Stutzen der SBM
- Gießen der überschüssigen Aufschlämmung in die Matrize, nachdem eine Aufschlämmungsschicht auf 10 mm verdickt wurde
- Zentrifugieren des Modells mit einem Rohling, nachdem die Aufschlämmung gegossen wurde
(5) Trocknen und Entformen:
- Platzieren des Modells mit einem Rohling, das in Schritt (4) erhalten wurde, in einem Trockenraum bei einer Temperatur von 53 +/- 3 °C
- Entformen des Modells mit einem Rohling, nachdem eine Vergussöffnung 0,5 bis 1 mm von dem Rohling getrennt ist
- dies erzeugt einen Rohling des Stutzens
(6) Vakuumsintern:
- Platzieren des Rohlings des Stutzens, der in Schritt (5) erhalten wurde, in einer Matrize des Stutzens
- Platzieren davon in einen Vakuum-Heißpress-Sinterofen mit einem Vakuumgrad von 10⁻² Pa
- Das Temperaturerhöhungsverfahren besteht aus:
- manuellem Erwärmen auf 200 °C
- Erwärmen auf 1100 °C bei einer Rate von 10 °C/Min
- Aufrechterhalten der Temperatur für 30 Min.
- Erwärmen auf 1750 bis 1800 °C bei einer Rate von 7 °C/Min
- Aufrechterhalten der Temperatur für 1 Std.
- dies erzeugt eine Verbundkeramikauskleidung des Stutzens aus Si₃N₄/BNNT, nachdem ein Werkstück in dem Ofen auf Raumtemperatur abgekühlt ist
(7) Verbundguss:
- Laden der Verbundkeramikauskleidung des Stutzens aus Si₃N₄/BNNT, die in Schritt (6) erhalten wurde, in eine Gusssandkiste des Stutzens
- Gießen von geschmolzenem Eisen nach der Matrizenmontage, um die Außenwand des Keramikstutzens mit einem Eisenguss zu umwickeln, wodurch schließlich der Verbundstutzen der SBM mit einer Außenseite aus Gusseisen und einer Innenseite aus Si₃N₄/BNNT-Verbundkeramik erhalten wird

2. Herstellungsverfahren für einen Verbundstutzen einer SBM nach Anspruch 1, **dadurch gekennzeichnet, dass** das Verdünnungsmittel in Schritt (3) ein oder eine Kombination aus mehreren von Wasserglas oder Natriumcarbonat oder Natriumphosphat oder Natriumhexametaphosphat ist.

3. Herstellungsverfahren für einen Verbundstutzen einer SBM nach Anspruch 2, **dadurch gekennzeichnet, dass** das Verdünnungsmittel Natriumcarbonat ist.

4. Herstellungsverfahren für einen Verbundstutzen einer SBM nach Anspruch 1, **dadurch gekennzeichnet, dass** die Trockenzeit für das Modell mit einem Rohling in Schritt (5) 2/5 bis 3/5 der Aufschlämmungsladezeit beträgt.

5. Herstellungsverfahren für einen Verbundstutzen einer SBM nach Anspruch 4, **dadurch gekennzeichnet, dass** die Trockenzeit für das Modell mit einem Rohling in Schritt (5) 1/2 der Aufschlämmungsladezeit beträgt.

6. Herstellungsverfahren für einen Verbundstutzen einer SBM nach Anspruch 1, umfassend die Schritte im Detail:
(1) Rohstoffaufbereitung:
- 80 Gewichtsteile Siliziumnitridpulver
- 10 Gewichtsteile Bornitrid-Nanoröhrenpulver
- 5 Gewichtsteile Aluminiumoxidpulver
- 5 Gewichtsteile Yttriumoxidpulver
(2) Rohstoffmischung:
- Zugeben der Rohstoffe aus Schritt (1) in einen Kugelmahlbehälter
- Hinzufügen von Alkohol gemäß einem Volumenverhältnis von Alkohol zu Rohstoffen von 1:1
- Hinzufügen von Stahlkies gemäß einem Massenverhältnis von Stahlkies zu Rohstoffen von 10:1
- Verschließen des Kugelmahlbehälters
- Einleiten von Argongas in den Kugelmahlbehälter als Schutzgas
- Kugelmahlen und Mischen der Rohstoffe in einer Planetenkugelmühle bei einer Rotationsgeschwindigkeit von 250 rpm, und einer Dauer von 10 Std.
- Trocknen der kugelgemahlenen Rohstoffe für 10 Std. in einem Vakuum-Trockner bei einer Temperatur von 75 °C
- Passieren der gemischten Materialen durch ein 300-maschiges Sieb nach dem Trocknen
(3) Aufschlämmungszubereitung:
- Zugeben des gemischten Materials, das in Schritt (2) erhalten wurde, in ein Rührgerät
- Hinzufügen von destilliertem Wasser mit einem Massenanteil von 30 %
- Hinzufügen von Wasserlösung mit einem Massenanteil von 0,3 %
- Rühren der Rohstoffe bei einer Rotationsgeschwindigkeit von 250 rpm für 1 Std.
(4) Vergussformung:
- Einspritzen der Aufschlämmung, die in Schritt (3) erhalten wurde, in eine Formteilgipsmatrize für den Stutzen der SBM
- Gießen der überschüssigen Aufschlämmung in die Matrize, nachdem eine Aufschlämmungsschicht auf 10 mm verdickt wurde
- Zentrifugieren des Modells mit einem Rohling, nachdem die Aufschlämmung gegossen wurde
(5) Trocknen und Entformen:
- Platzieren des Modells mit einem Rohling, das in Schritt (4) erhalten wurde, in einem Trockenraum bei einer Temperatur von 53 +/- 3 °C
- Entformen des Modells mit einem Rohling, nachdem eine Vergussöffnung 1 mm von dem Rohling getrennt ist, um einen Rohling des Kugelflussrohrs zu erhalten
- die Trockenzeit des Modells mit einem Rohling beträgt 3/5 der Aufschlämmungsladungszeit
(6) Vakuumsintern:
- Platzieren des Rohlings des Stutzens, der in Schritt (5) erhalten wurde, in einer Matrize des Stutzens
- Platzieren davon in einen Vakuum-Heißpress-Sinterofen mit einem Vakuumgrad von 10⁻² Pa, und ein Temperaturerhöhungsverfahren, bestehend aus:
- manuellem Erwärmen auf 200 °C
- Erwärmen auf 1100 °C bei einer Rate von 10 °C/Min
- Aufrechterhalten der Temperatur für 30 Min.
- Erwärmen auf 1750°C bei einer Rate von 7 °C/Min
- Aufrechterhalten der Temperatur für 1 Std.
- dies führt zum Erhalt einer Verbundkeramikauskleidung des Stutzens aus Si₃N₄/BNNT, nachdem das Werkstück in dem Ofen auf Raumtemperatur abgekühlt ist
(7) Verbundguss:
- Laden der Verbundkeramikauskleidung des Stutzens aus Si₃N₄/BNNT, die in Schritt (6) erhalten wurde, in eine Gusssandkiste des Stutzens
- Gießen mit geschmolzenem Eisen nach der Matrizenmontage, um einen Eisenguss um die Außenwand des Keramikstutzens zu wickeln
- dadurch wird der Verbundstutzen der SBM mit der Außenseite aus Gusseisen und der Innenseite aus Si₃N₄/BNNT-Verbundkeramik erhalten.

7. Herstellungsverfahren für einen Verbundstutzen einer SBM nach Anspruch 1, umfassend die Schritte im Detail:
(1) Rohstoffaufbereitung:
- 82 Gewichtsteile Siliziumnitridpulver
- 8 Gewichtsteile Bornitrid-Nanoröhrenpulver
- 6 Gewichtsteile Aluminiumoxidpulver
- 4 Gewichtsteile Yttriumoxidpulver
(2) Rohstoffmischung:
- Zugeben der Rohstoffe aus Schritt (1) in einen Kugelmahlbehälter
- Hinzufügen von Alkohol gemäß einem Volumenverhältnis von Alkohol zu Rohstoffen von 1:1
- Hinzufügen von Stahlkies gemäß einem Massenverhältnis von Stahlkies zu Rohstoffen von 9:1
- Verschließen des Kugelmahlbehälters
- Einleiten von Argongas in den Kugelmahlbehälter als Schutzgas
- Kugelmahlen und Mischen der Rohstoffe in der Planetenkugelmühle bei einer Rotationsgeschwindigkeit von 250 rpm, und einer Dauer von 8 Std.
- Trocknen der kugelgemahlenen Rohstoffe für 12 Std. in einem Vakuum-Trockner bei einer Temperatur von 85°C
- Passieren der gemischten Materialen durch ein 300-maschiges Sieb nach dem Trocknen
(3) Aufschlämmungszubereitung:
- Zugeben des gemischten Materials, das in Schritt (2) erhalten wurde, in ein Rührgerät
- Hinzufügen von destilliertem Wasser mit einem Massenanteil von 32 %
- Hinzufügen von Natriumcarbonat mit einem Massenanteil von 0,4 %
- Rühren der Rohstoffe bei einer Rotationsgeschwindigkeit von 250 rpm für 1,5 Std.
(4) Vergussformung:
- Einspritzen der Aufschlämmung, die in Schritt (3) erhalten wurde, in eine Formteilgipsmatrize für den Stutzen der SBM
- Gießen der überschüssigen Aufschlämmung in die Matrize, nachdem eine Aufschlämmungsschicht auf 10 mm verdickt wurde
- Zentrifugieren des Modells mit einem Rohling, nachdem die Aufschlämmung gegossen wurde
(5) Trocknen und Entformen:
- Platzieren des Modells mit einem Rohling, das in Schritt (4) erhalten wurde, in einem Trockenraum bei einer Temperatur von 53 +/- 3 °C
- Entformen des Modells mit einem Rohling, nachdem eine Vergussöffnung 1 mm von dem Rohling getrennt ist, was einen Rohling des Stutzens erzeugt
- die Trockenzeit des Modells mit einem Rohling beträgt 1/2 der Aufschlämmungsladungszeit
(6) Vakuumsintern:
- Platzieren des Rohlings des Stutzens, der in Schritt (5) erhalten wurde, in einer Matrize des Stutzens
- Platzieren davon in einen Vakuum-Heißpress-Sinterofen bei einem Vakuumgrad von 10⁻² Pa
- Das Temperaturerhöhungsverfahren besteht aus:
- manuellem Erwärmen auf 200 °C
- Erwärmen auf 1100 °C bei einer Rate von 10 °C/Min
- Aufrechterhalten der Temperatur für 30 Min.
- Erwärmen auf 1780 °C bei einer Rate von 7 °C/Min
- Aufrechterhalten der Temperatur für 1 Std.
- dies führt zum Erhalt einer Verbundkeramikauskleidung des Stutzens aus Si₃N₄/BNNT, nachdem das Werkstück in dem Ofen auf Raumtemperatur abgekühlt ist
(7) Verbundguss:
- Laden der Verbundkeramikauskleidung des Stutzens aus Si₃N₄/BNNT, die in Schritt (6) erhalten wurde, in eine Gusssandkiste des Stutzens
- Gießen mit geschmolzenem Eisen nach der Matrizenmontage, um einen Eisenguss um die Außenwand des Keramikstutzens zu wickeln
- dadurch wird der Verbundstutzen der SBM mit der Außenseite aus Gusseisen und der Innenseite aus Si₃N₄/BNNT-Verbundkeramik erhalten.

8. Herstellungsverfahren für einen Verbundstutzen einer SBM nach Anspruch 1, umfassend die Schritte im Detail:
(1) Rohstoffaufbereitung:
- 85 Gewichtsteile Siliziumnitridpulver
- 5 Gewichtsteile Bornitrid-Nanoröhrenpulver
- 4 Gewichtsteile Aluminiumoxidpulver
- 3 Gewichtsteile Yttriumoxidpulver
(2) Rohstoffmischung:
- Zugeben der Rohstoffe aus Schritt (1) in einen Kugelmahlbehälter
- Hinzufügen von Alkohol gemäß einem Volumenverhältnis von Alkohol zu Rohstoffen von 1:1
- Hinzufügen von Stahlkies gemäß einem Massenverhältnis von Stahlkies zu Rohstoffen von 15:1
- Verschließen des Kugelmahlbehälters
- Einleiten von Argongas in den Kugelmahlbehälter als Schutzgas
- Kugelmahlen und Mischen der Rohstoffe in einer Planetenkugelmühle mit einer Rotationsgeschwindigkeit von bis 200 rpm für eine Dauer von 12 Std.
- Trocknen der kugelgemahlenen Rohstoffe für 12 Std. in einem Vakuum-Trockner bei einer Temperatur von 75 °C
- Passieren der gemischten Materialen durch ein 300-maschiges Sieb nach dem Trocknen
(3) Aufschlämmungszubereitung:
- Zugeben des gemischten Materials, das in Schritt (2) erhalten wurde, in ein Rührgerät
- Hinzufügen von destilliertem Wasser mit einem Massenanteil von 35 %
- Hinzufügen einer Kombination aus Natriumphosphat und Natriumhexametaphosphat mit einem Massenanteil von 0,5 %, und wobei das Massenverhältnis von Natriumphosphat zu Natriumhexametaphosphat 1:1 beträgt
- Rühren der Rohstoffe bei einer Rotationsgeschwindigkeit von 300 rpm für eine Dauer von 1 Std.
(4) Vergussformung:
- Einspritzen der Aufschlämmung, die in Schritt (3) erhalten wurde, in eine Formteilgipsmatrize für den Stutzen der SBM
- Gießen der überschüssigen Aufschlämmung in die Matrize, nachdem eine Aufschlämmungsschicht auf 10 mm verdickt wurde
- Zentrifugieren des Modells mit einem Rohling, nachdem die Aufschlämmung gegossen wurde
(5) Trocknen und Entformen:
- Platzieren des Modells mit einem Rohling, das in Schritt (4) erhalten wurde, in einem Trockenraum bei einer Temperatur von 53 +/- 3 °C
- Entformen des Modells mit einem Rohling, nachdem eine Vergussöffnung 1 mm von dem Rohling getrennt ist, um einen Rohling des Stutzens zu erhalten
- die Trockenzeit des Modells mit einem Rohling beträgt 2/5 der Aufschlämmungsladungszeit
(6) Vakuumsintern:
- Platzieren des Rohlings des Stutzens, der in Schritt (5) erhalten wurde, in einer Matrize des Stutzens
- Platzieren davon in einem Vakuum-Heißpress-Sinterofen, wobei der Vakuumgrad 10⁻² Pa beträgt
- Das Temperaturerhöhungsverfahren besteht aus:
- manuellem Erwärmen auf 200 °C
- Erwärmen auf 1100 °C bei einer Rate von 10 °C/Min
- Aufrechterhalten der Temperatur für 30 Min.
- Erwärmen auf 1800 °C bei einer Rate von 7 °C/Min
- Aufrechterhalten der Temperatur für 1 Std.
- dies führt zum Erhalt einer Verbundkeramikauskleidung des Kugelflussrohrs aus Si₃N₄/BNNT, nachdem ein Werkstück in dem Ofen auf Raumtemperatur abgekühlt ist
(7) Verbundguss:
- Laden der Verbundkeramikauskleidung des Stutzens aus Si₃N₄/BNNT, die in Schritt (6) erhalten wurde, in eine Gusssandkiste des Stutzens
- Gießen mit geschmolzenem Eisen nach der Matrizenmontage, um einen Eisenguss um die Außenwand des Keramikstutzens zu wickeln
- dadurch wird der Verbundstutzen der SBM mit der Außenseite aus Gusseisen und der Innenseite aus Si₃N₄/BNNT-Verbundkeramik erhalten.

## Revendications

1. Procédé de préparation d'un goulot composite d'un SBM comprenant les étapes suivantes :
(1) Préparation de matière brute :
- 80 à 85 parties en poids de poudre de nitrure de silicium
- 5 à 10 parties en poids de poudre de nanotube de nitrure de bore
- 4 à 6 parties en poids de poudre d'oxyde d'aluminium
- 3 à 5 parties en poids de poudre d'oxyde d'yttrium
(2) mélange des matières brutes :
- ajouter les matières brutes dans l'étape (1) dans une cuve de broyage à boule
- ajouter de l'alcool selon un rapport en volume d'alcool à matières brutes de 1 : 1
- ajouter de la grenaille d'acier selon un rapport en masse de la grenaille d'acier aux matières brutes de 9 à 15 : 1
- sceller la cuve de broyage à boule
- introduire du gaz argon dans la cuve de broyage à boule comme gaz protecteur
- broyer avec les boules et mélanger les matières brutes dans un broyeur à boule planétaire avec une vitesse de rotation de 200 à 250 tpm et une durée de 8 à 12 h
- sécher les matières brutes broyées par boule durant 10 à 12 heures dans une boîte de séchage sous vide à une température de 75 à 85 °C
- passer les matières mélangées après le séchage à travers un tamis de maille 300
(3) préparation de solution épaisse :
- ajouter la matière mélangée obtenue dans l'étape (2) dans une machine d'agitation
- ajouter de l'eau distillée avec un pourcentage en masse de 28 à 35 %
- ajouter un diluant avec un pourcentage en masse de 0,3 à 0,5 %
- agiter les matières brutes à une vitesse de rotation de 250 à 300 t/min durant 1 à 2 h
(4) moulage par scellement :
- injecter la solution épaisse obtenue dans l'étape (3) dans un moule de gypse de moulage pour le goulot du SBM
- verser la solution épaisse en excès dans le moule après qu'une couche de solution épaisse soit épaissie à 10 mm
- centrifuger le modèle avec un témoin après le versement de la solution épaisse
(5) démoulage par séchage :
- placer le modèle avec un témoin obtenu dans l'étape (4) dans une chambre de séchage à une température de 53 ± 3 °C
- démouler le modèle avec un témoin après qu'une ouverture de scellement est séparée du témoin par 0,5 à 1 mm
- cela résulte dans un témoin du goulot
(6) frittage sous vide
- placer le témoin du goulot obtenu dans l'étape (5) dans un moule du goulot
- le placer dans un four de frittage à pression thermique sous vide avec un degré de vide de 10⁻² Pa
- le processus d'augmentation de la température consiste en :
- chauffage manuel à 200 °C
- chauffer à 1100 °C à une vitesse de 10 °C/min
- maintenir la température durant 30 minutes
- chauffer à 1750 à 1800 °C à une vitesse de 7 °C/min
- maintenir la température durant 1 h
- cela résulte dans un revêtement en céramique composite de Si₃N₄/BNNT du goulot après qu'un outil est refroidi à température ambiante dans le four
(7) moulage de composite :
- charger le revêtement en céramique composite Si₃N₄/BNT du goulot obtenu dans l'étape (6) dans une sablière de moulage du goulot
- verser du fer fondu après l'assemblage du moule pour envelopper un moulage de fer sur la paroi externe du goulot en céramique, obtenant finalement ainsi le goulot composite du SBM avec le côté externe du fer moulé et à l'intérieur la céramique composite de Si₃N₄/BNNT.

2. Procédé de préparation d'u goulot composite d'un SBM selon la revendication 1, **caractérisé en ce que** le diluant dans l'étape (3) est un ou une combinaison de plusieurs de verre d'eau ou de carbonate de sodium ou de phosphate de sodium ou d'hexamétaphosphate de sodium.

3. Procédé de préparation d'un goulot composite d'un SBM selon la revendication 2, **caractérisé en ce que** le diluant est le carbonate de sodium.

4. Procédé de préparation d'un goulot composite de SBM selon la revendication 1, **caractérisé en ce que** le temps de séchage pour le modèle avec un témoins dans l'étape (5) est de 2/5 à 3/5 du temps de chargement de solution épaisse.

5. Procédé de préparation d'un goulot composite de SBM selon la revendication 4, **caractérisé en ce que** le temps de séchage pour le modèle avec un témoin dans l'étape (5) est 1/2 du temps de chargement de solution épaisse.

6. Procédé de préparation d'un goulot composite de SBM selon la revendication 1, comprenant les étapes en détail :
(1) préparation des matières brutes :
- 80 parties en poids de poudre de nitrure de silicium
- 10 parties en poids de poudre de nanotube de nitrure de bore
- 5 parties en poids de poudre d'oxyde d'aluminium
- 5 parties en poids de poudre d'oxyde d'yttrium
(2) mélange des matières brutes
- ajouter les matières brutes dans l'étape (1) dans une cuve de broyage à boule
- ajouter de l'alcool selon un rapport en volume d'alcool à matières brutes de 1 : 1
- ajouter de la grenaille d'acier selon un rapport en masse de la grenaille d'acier aux matières brutes de 10 : 1
- sceller la cuve de broyage à boule
- introduire du gaz argon dans la cuve de broyage à boule comme gaz protecteur
- broyer avec les boules et mélanger les matières brutes dans un broyeur à boule planétaire avec une vitesse de rotation de 250 tpm avec une durée de 10 h
- sécher les matières brutes broyées par boule durant 10 h dans un boîte de séchage sous vide à une température de 75 °C
- passer les matières mélangées après le séchage à travers un tamis de maille 300
(3) préparation de la solution épaisse :
- ajouter la matière mélangée obtenue dans l'étape (2) dans une machine d'agitation
- ajouter de l'eau distillée avec un pourcentage en masse de 30 %
- ajouter une solution d'eau avec un pourcentage en masse de 0,3 %
- agiter les matières brutes à une vitesse de rotation de 250 t/min durant 1 h
(4) moulage par scellement :
- injecter la solution épaisse obtenue dans l'étape (3) dans un moule de gypse de moulage pour le goulot du SBM
- verser la solution épaisse en excès dans le moule après qu'une couche de solution épaisse soit épaissie à 10 mm
- centrifuger le modèle avec un témoin après le versement de la solution épaisse
(5) démoulage par séchage :
- placer le modèle avec un témoin obtenu dans l'étape (4) dans une chambre de séchage à une température de 53 ± 3 °C
- démouler le modèle avec un témoin après qu'une ouverture de scellement est séparée du témoin par 1 mm pour obtenir un témoin du tube d'écoulement de grenaille
- le temps de séchage du modèle avec un témoin est 3/5 du temps de chargement de solution épaisse
(6) frittage sous vide :
- placer le témoin du goulot obtenu dans l'étape (5) dans un moule du goulot
- le placer dans un four de frittage à pression thermique sous vide avec un degré de vide de 10⁻² Pa et un processus d'augmentation de la température consistant en :
- chauffage manuel à 200 °C
- chauffer à 1100 °C à une vitesse de 10 °C/min
- maintenir la température durant 30 minutes
- chauffer à 1750 °C à une vitesse de 7 °C/min
- maintenir la température durant 1 h
- cela résulte dans un revêtement en céramique composite de Si₃N₄/BNNT du goulot après qu'un outil est refroidi à température ambiante dans le four
(7) moulage de composite :
- charger le revêtement en céramique composite Si₃N₄/BNT du goulot obtenu dans l'étape (6) dans une sablière de moulage du goulot
- verser du fer fondu après l'assemblage du moule pour envelopper le moulage de fer sur la paroi externe du goulot en céramique
- cela résulte dans l'obtention du goulot composite du SBM avec le côté externe du fer moulé et à l'intérieur la céramique composite de Si₃N₄/BNNT

7. Procédé de préparation d'un goulot composite d'un WBM selon la revendication 1 comprenant les étapes en détail :
(1) préparation des matières brutes :
- 82 parties en poids de poudre de nitrure de silicium
- 8 parties en poids de poudre de nanotube de nitrure de bore
- 6 parties en poids de poudre d'oxyde d'aluminium
- 4 parties en poids de poudre d'oxyde d'yttrium
(2) mélange des matières brutes :
- ajouter les matières brutes dans l'étape (1) dans une cuve de broyage à boule
- ajouter de l'alcool selon un rapport en volume d'alcool à matières brutes de 1 : 1
- ajouter de la grenaille d'acier selon un rapport en masse de la grenaille d'acier aux matières brutes de 9 : 1
- sceller la cuve de broyage à boule
- introduire du gaz argon dans la cuve de broyage à boule comme gaz protecteur
- broyer avec les boules et mélanger les matières brutes dans un broyeur à boule planétaire avec une vitesse de rotation de 250 tpm pour une durée de 8 h
- sécher les matières brutes broyées par boule durant 12 h dans une boîte de séchage sous vide à une température de 85 °C
- passer les matières mélangées après le séchage à travers un tamis de maille 300
(3) préparation de la solution épaisse :
- ajouter la matière mélangée obtenue dans l'étape (2) dans une machine d'agitation
- ajouter de l'eau distillée avec un pourcentage en masse de 32 %
- ajouter du carbonate de sodium avec un pourcentage en masse de 0,4 %
- agiter les matières brutes à une vitesse de rotation de 250 t/min durant 1,5 h
(4) moulage par scellement
- injecter la solution épaisse obtenue dans l'étape (3) dans un moule de gypse de moulage pour le goulot du SBM
- verser la solution épaisse en excès dans le moule après qu'une couche de solution épaisse soit épaissie à 10 mm
- centrifuger le modèle avec un témoin après le versement de la solution épaisse
(5) démoulage par séchage :
- placer le modèle avec un témoin obtenu dans l'étape (4) dans une chambre de séchage à une température de 53 ± 3 °C
- démouler le modèle avec un témoin après qu'une ouverture de scellement est séparée du témoin par 1 mm qui résulte dans un témoin du goulot
- le temps de séchage du modèle avec un témoin est 1/2 du temps de chargement de solution épaisse
(6) frittage sous vide :
- placer le témoin du goulot obtenu dans l'étape (5) dans un moule du goulot
- le placer dans un four de frittage à pression thermique sous vide avec un degré de vide de 10⁻² Pa
- le processus d'augmentation de la température consiste en :
- chauffage manuel à 200 °C
- chauffer à 1100 °C à une vitesse de 10 °C/min
- maintenir la température durant 30 minutes
- chauffer à 1780 °C à une vitesse de 7 °C/min
- maintenir la température durant 1 h
- cela résulte dans l'obtention d'un revêtement en céramique composite de Si₃N₄/BNNT du goulot après que l'outil est refroidi à température ambiante dans le four
(7) moulage de composite :
- charger le revêtement en céramique composite Si₃N₄/BNNT du goulot obtenu dans l'étape (6) dans une sablière de moulage du goulot
- verser du fer fondu après l'assemblage du moule pour envelopper le moulage de fer sur la paroi externe du goulot en céramique
- cela résulte dans l'obtention du goulot composite du SBM avec le côté externe du fer moulé et à l'intérieur la céramique composite de Si₃N₄/BNNT.

8. Procédé de préparation d'un goulot composite d'un SBM selon la revendication 1, comprenant les étapes en détail :
(1) Préparation des matières brutes :
- 85 parties en poids de poudre de nitrure de silicium
- 5 parties en poids de poudre de nanotube de nitrure de bore
- 4 parties en poids de poudre d'oxyde d'aluminium
- 3 parties en poids de poudre d'oxyde d'yttrium
(2) mélange des matières brutes :
- ajouter les matières brutes dans l'étape (1) dans une cuve de broyage à boule
- ajouter de l'alcool selon un rapport en volume d'alcool à matières brutes de 1 : 1
- ajouter de la grenaille d'acier selon un rapport en masse de la grenaille d'acier aux matières brutes de 15 : 1
- sceller la cuve de broyage à boule
- introduire du gaz argon dans la cuve de broyage à boule comme gaz protecteur
- broyer avec les boules et mélanger les matières brutes dans un broyeur à boule planétaire avec une vitesse de rotation de 200 tpm pour une durée de 12 h
- sécher les matières brutes broyées par boule durant 12 h dans une boîte de séchage sous vide à une température de 75 °C
- passer les matières mélangées après le séchage à travers un tamis de maille 300
(3) préparation de la solution épaisse :
- ajouter la matière mélangée obtenue dans l'étape (2) dans une machine d'agitation
- ajouter de l'eau distillée avec un pourcentage en masse de 35 %
- ajouter une combinaison de phosphate de sodium et d'hexamétaphosphate de sodium avec un pourcentage en masse de 0,5 % et où le rapport en masse du phosphate de sodium à l'hexamétaphosphate de sodium est de 1 : 1
- agiter les matières brutes à une vitesse de rotation de 300 t/min durant 1 h
(4) moulage par scellement :
- injecter la solution épaisse obtenue dans l'étape (3) dans un moule de gypse de moulage pour le goulot du SBM
- verser la solution épaisse en excès dans le moule après qu'une couche de solution épaisse soit épaissie à 10 mm
- centrifuger le modèle avec un témoin après le versement de la solution épaisse
(5) démoulage par séchage :
- placer le modèle avec un témoin obtenu dans l'étape (4) dans une chambre de séchage à une température de 53 ± 3 °C
- démouler le modèle avec un témoin après qu'une ouverture de scellement est séparée du témoin par 1 mm qui résulte dans un témoin du goulot
- le temps de séchage du modèle avec un témoin est 2/5 du temps de chargement de solution épaisse
(6) frittage sous vide :
- placer le témoin du goulot obtenu dans l'étape (5) dans un moule du goulot
- le placer dans un four de frittage à pression thermique sous vide avec un degré de vide de 10⁻² Pa
- le processus d'augmentation de la température consiste en :
- chauffage manuel à 200 °C
- chauffer à 1100 °C à une vitesse de 10 °C/min
- maintenir la température durant 30 minutes
- chauffer à 1800 °C à une vitesse de 7 °C/min
- maintenir la température durant 1 h
- cela résulte dans l'obtention d'un revêtement en céramique composite de Si₃N₄/BNNT du tube d'écoulement de grenaille après qu'un outil est refroidi à température ambiante dans le four
(7) moulage de composite
- charger le revêtement en céramique composite Si₃N₄/BNNT du goulot obtenu dans l'étape (6) dans une sablière de moulage du goulot
- verser du fer fondu après l'assemblage du moule pour envelopper le moulage de fer sur la paroi externe du goulot en céramique
- cela résulte dans l'obtention du goulot composite du SBM avec le côté externe du fer moulé et à l'intérieur la céramique composite de Si₃N₄/BNNT.
